

## UNITED STATES PATENT OFFICE

2,436,690

ACID CHLORIDE-FLUORIDE BATH FOR  
NICKEL PLATING

Arthur H. Du Rose, Euclid, Ohio, assignor to The  
Harshaw Chemical Company, Elyria, Ohio, a  
corporation of Ohio

No Drawing. Application March 12, 1945,  
Serial No. 582,423

3 Claims. (Cl. 204—49)

2

**1**  
This invention relates to electrodeposition of nickel from "high chloride" solutions, and more particularly a chloride-fluoride bath omitting boric acid.

I have now discovered that the use of certain fluorides in nickel plating solutions of the high chloride type instead of the usual boric acid buffer is advantageous in respect to ductility of the resulting deposit, throwing power and freedom from pitting. The solution also remains clear at pH values above 5.0 whereas the usual bath buffered with boric acid becomes turbid. There is also a slight increase in brightness in the all chloride solution and solutions in which the nickel in solution is more than half derived from chloride.

By "high chloride" solutions I mean those in which at least 33 1/3 % of the nickel is from chloride, the remainder from sulfate.

As is well known, all-chloride nickel plating solutions normally yield more highly stressed deposits than do solutions high in sulfate. With the advent of equipment suitable for containing the all-chloride solution there has been substantial tendency in the last few years for workers in the art of nickel plating to experiment with solutions of the all-chloride or high-chloride type in an attempt to produce deposits no more highly stressed than those taken from the usual high-sulfate solutions. Surprisingly, the use of fluorides as described below results in marked reduction in stress in the deposit. For example, a half chloride bath using fluorides gives a deposit which is no more highly stressed than those derived from the normal high-sulfate bath. This comparison is between solutions buffered with fluoride on the one hand and with boric acid on the other, 15 to 30 grams per liter of NH<sub>4</sub>HF<sub>2</sub> or equivalent fluorine content of other fluorides as described below compared with 37.5 grams per liter of boric acid in standard Watts bath, these being optimum concentrations in both cases. Still more surprisingly, the use of fluorides as described below gives improved results in respect to throwing power, pitting, brightness and buffering action.

Fluorides suitable for my purpose are HF, NaF, KHF<sub>2</sub>, NH<sub>4</sub>HF<sub>2</sub>, NiF<sub>2</sub>, and NiHF. These are used in quantity between 15 and 30 grams per liter in the case of NH<sub>4</sub>HF<sub>2</sub> and in the other cases the

equivalent in fluorine content of 15 to 30 grams per liter of NH<sub>4</sub>HF<sub>2</sub>.

Suitable bath compositions are as follows:

5 Nickel chloride hexahydrate 33 1/3 % to 100%—grams per liter... 200 to  
Nickel sulfate hexahydrate 66 2/3 % to 0%—do— 400  
A substance of the class consisting of NH<sub>4</sub>HF<sub>2</sub>, HF, NaF, KHF<sub>2</sub>, NiF<sub>2</sub>, and NiHF and mixtures of a plurality thereof, the total fluorine content thereof being equivalent to NH<sub>4</sub>HF<sub>2</sub>—grams per liter... 15 to 30  
Water—do—Remainder  
pH (may be adjusted with HCl)— 2.5 to 5.5

10 10 Specific examples of preferred bath proportions according to the invention are as follows:

*Example I*

|    |                                      |       |      |
|----|--------------------------------------|-------|------|
| 15 | NiCl <sub>2</sub> .6H <sub>2</sub> O | grams | 250  |
| 15 | NH <sub>4</sub> HF <sub>2</sub>      | do    | 20   |
|    | Water to make                        | ml    | 1000 |

*Example II*

|    |                                      |       |      |
|----|--------------------------------------|-------|------|
| 20 | NiCl <sub>2</sub> .6H <sub>2</sub> O | grams | 150  |
| 20 | NiSO <sub>4</sub> .6H <sub>2</sub> O | do    | 150  |
|    | NH <sub>4</sub> HF <sub>2</sub>      | do    | 15   |
|    | Water to make                        | ml    | 1000 |

*Example III*

|    |                                      |       |      |
|----|--------------------------------------|-------|------|
| 25 | NiCl <sub>2</sub> .6H <sub>2</sub> O | grams | 250  |
|    | NaF                                  | do    | 12   |
|    | Water to make                        | ml    | 1000 |

*Example IV*

|    |                                      |       |      |
|----|--------------------------------------|-------|------|
| 30 | NiCl <sub>2</sub> .6H <sub>2</sub> O | grams | 150  |
|    | NiSO <sub>4</sub> .6H <sub>2</sub> O | do    | 150  |
|    | NaF                                  | do    | 20   |
|    | Water to make                        | ml    | 1000 |

Having thus described my invention, what I claim is:

1. A nickel plating solution essentially consisting of water from 200 to 400 grams per liter of a source of nickel of the class consisting of (1) nickel chloride and (2) nickel chloride plus nickel sulfate, in proportion such that at least 33 1/3 % of the nickel is from the chloride, HCl sufficient to produce a pH of from 2.5 to 5, and a source of fluorine of the class consisting of NH<sub>4</sub>HF<sub>2</sub>, HF, NaF, KHF<sub>2</sub>, NiF<sub>2</sub>, NiHF and mixtures of a plurality thereof, the total fluorine content of said source of fluorine being equivalent to from 15 to 30 grams per liter of NH<sub>4</sub>HF<sub>2</sub>.

2. A nickel plating solution essentially consisting of water, nickel chloride, HCl sufficient to produce a pH of from 2.5 to 5, and from 15 to 30

grams per liter of a substance of the class consisting of  $\text{NH}_4\text{HF}_2$ , HF, NaF,  $\text{KHF}_2$ ,  $\text{NiF}_2$ ,  $\text{NiHF}$  and mixtures of a plurality thereof.

3. A nickel plating solution essentially consisting of water, from 200 to 400 grams per liter of a source of nickel of the class consisting of (1) nickel chloride and (2) nickel chloride plus nickel sulfate in proportion that at least 50% of the nickel is from the chloride, HCl in quantity sufficient to produce a pH of 2.5 to 5, and a source of fluorine of the class consisting of  $\text{NH}_4\text{HF}_2$ , HF, NaF,  $\text{KHF}_2$ ,  $\text{NiF}_2$ ,  $\text{NiHF}$  and mixtures of a plurality thereof, the total fluorine content of said source of fluorine being equivalent to from 15 to 30 grams per liter of  $\text{NH}_4\text{HF}_2$ .

ARTHUR H. DU ROSE.

REFERENCES CITED

The following references are of record in the file of this patent:

UNITED STATES PATENTS

|           |       |               |
|-----------|-------|---------------|
| Number    | Name  | Date          |
| 2,313,756 | Loose | Mar. 16, 1943 |

FOREIGN PATENTS

|         |               |               |
|---------|---------------|---------------|
| Number  | Country       | Date          |
| 513,963 | Great Britain | Oct. 26, 1939 |

OTHER REFERENCES

Transactions of the Electrochemical Society, vol. 75 (1939), pages 209-211, by W. A. Wesley et al.

10 Transactions of the American Electrochemical Society, vol. (XLXI) (1922), pages 344-346, by M. R. Thompson.

Transactions of the Faraday Society, vol. 31, (1935), pages 1203 to 1205 and 1208-1210. (An 15 article by W. Blum et al.)

Electro-Plating by S. Field et al., published by I. Pitman and Sons, London 1930, pages 118 and 130.

20 Nickel and Its Alloys, Circular of Bureau of Standards, No. 100 (1924), page 50.